# EUROPEAN PATENT SPECIFICATION

(11) **EP 0 199 567 B1**
(45) Date of publication and mention of the grant of the patent: **26.08.1992**
(21) Application number: 86302959.1
(22) Date of filing: 18.04.1986
(51) Int. Cl.: D01F 9/22, D01F 9/14, D01F 9/20

(54) **Carbonaceous fibers with spring-like reversible deflection and method of manufacture**
Kohlenstoffartige Faser mit federartiger umkehrbarer Abbiegung und Verfahren zur Herstellung
Fibres du genre carbone ayant des propriétés de déflexion réversible comme un ressort et méthode de préparation

(30) Priority: 18.04.1985 US 724440; 10.02.1986 US 827567
(43) Date of publication of application: 29.10.1986
(73) Proprietor: THE DOW CHEMICAL COMPANY, Midland Michigan 48640-1967 (US)
(72) Inventor: McCullough, Francis Patrick, Jr., Lake Jackson Texas 77566 (US); Hall, David Michael, Auburn Alabama 36830 (US)
(74) Representative: Burford, Anthony Frederick

(56) References cited:
- FR-A- 1 539 755
- US-A- 4 351 816
- US-A- 4 412 675
- CHEMICAL ABSTRACTS, vol. 98, 1983, page 81, abstract no. 144959r, Columbus, Ohio, US; & JP-A-57 175 664 (MURATA MACHINERY, LTD) 28-10-1982

## Description

The invention resides in a carbonaceous resilient fiber or fiber assembly derived from a stabilized carbonaceous precursor material having imparted thereto a spring-like structural configuration capable of reversible deflection of greater than 1.2 times the length of the fiber when in a relaxed condition.

The carbonaceous fiber of the present invention is provided with a substantially permanent, non-linear, resilient, elongatable, spring-like structural configuration, e.g. of a substantial coil-like, sinusoidal or other multi-curvilinear configuration having no sharp or acute angular bends in the fiber. The spring-like structural configuration and the resilient, elongatable, characteristics of the fiber allows for a dimensional change of the fiber from a relaxed condition (ie. spring-like configuration) to an elongated, stretched, and substantially linear state, or any degree there-in-between, in which the fiber is under tension. When placed under tension, the fiber can be extended at least 1.2 times, typically from 2 to 4 times, the length of the fiber in its relaxed non-deflected spring-like configuration. The spring-like fiber can thus be deflected (elongated or stretched) to a substantially linear shape or configuration. If the modulus of elasticity of the fiber per se is not approached or exceeded, that is to say the fiber is not put under tension beyond that necessary to straighten the fiber to a substantially linear shape, the fiber is capable of returning from the linear to its relaxed spring-like shape over many cycles of stress elongation and relaxation without either breaking or substantially altering the dimensions or physical structure of the fiber.

The prior art has generally taught the manufacture of filaments from pitch based (petroleum and/or coal tar) compositions by the conventional technique of melt spinning the composition into continuous filaments which can then be stabilized by oxidation. Such filaments are taught to be useful per se. Alternatively, the continuous filament may be chopped or stretch-broken into what the art refers to as a "staple" fiber. Such "staple" fiber can be converted into a yarn by drafting, drawing and twisting, (referred to as spinning in the industry). The continuous filaments can also be made into a tow formed from a plurality of continuous mono-filaments. The resulting yarn or threads are used per se or may be woven into cloth-like articles and used as such. Alternatively, a woven article may be carbonized to produce a graphite or graphite-like cloth. In addition, a tow per se, may be carbonized, without weaving the tow into a cloth, and thereafter used as a reinforcement material for synthetic resinous materials e.g. "pre-preg", and the like.

In a somewhat similar manner it has been taught that polyacrylonitrile (PAN) can be wet spun into filaments; the filaments assembled into filament tow; the filaments or tow stabilized by oxidation; the filaments or tow made into staple by chopping or stretch breaking; the staple spun into yarn; the yarn knitted or woven into a cloth or fabric; and, if desired, the resulting fabric carbonized at a temperature of greater than 1400°C. These materials, in their pre-carbonized woven state, have been used as a non-combustible reinforcing material for metallized fire fighting suits. In their unwoven carbonized form, these materials have also been used as a reinforcement material for synthetic resinous materials such as golf club shafts, and the like.

In preparing uncarbonized conventional polymeric textile yarns for knitting, weaving or other textile manufacture, it is the usual practice in the industry to pinch crimp a fiber tow and thus sharply crimp-set the individual fibers of the tow (placing sharp or acute angular bends into the fiber). Such textile treatment has the same effect if used on a stabilized carbonaceous precursor yarn, i.e. severe and sharp angular crimps are imparted to the yarn causing entanglement among the individual fibers of the yarn and thus assisting in maintaining or fixing the short staple fibers in the yarn as well as imparting bulk properties to the yarn. However, when the procedure for the manufacture of ordinary textile yarn is followed and a yarn made from a carbonaceous precursor material is crimped and then carbonized, usually at a temperature above about 1000°C and, more practically, at a temperature of 1400°C and above, the resulting carbonized yarn becomes very brittle. That is to say, the yarn cannot be harshly handled or sharply creased, e.g. knitted or woven unless the knitting or weaving is done with great care and under highly controlled processing conditions. By the same token, such a knitted or woven yarn cannot be readily deknitted, garnetted or carded without breaking the fibers in the yarn into small segments. As a result of such brittleness, a knitted fabric cannot be deknitted without special care and such a deknitted yarn cannot thereafter be carded to convert the fibers in the yarn into a wool-like fluffy material without causing severe destruction, i.e. breakage, of the fibers. The resulting short and broken fibers do not have sufficient length or crimp to produce a well entangled fluff.

The prior art also generally discloses carbonized filaments having a high tensile strength or a high surface area. Such filaments are of a highly "graphitic" nature and necessitate the utilization of high temperatures to obtain a high degree of carbonization. However, the filaments produced by such a high temperature treatment are very brittle and incapable of standing up to stress such as repeated bending of the filaments, particularly when they have been subjected to a temperature above about 1000°C, and more so when they have been subjected to a temperature of above about 1400°C. Exemplary of a high temperature treatment of filaments derived from stabilized mesophase pitch can be found in U.S. Patent No. 4,005,183 where the oxidation stabilized (at a temperature of from 250° to 400°C) fibers are made into a yarn having a low (below normal absorptive carbon) surface area and a Young's modulus within the range of from 1 to 55 million psi (7 - 380 GPa).

Another technique for making a fabric panel is described in U.S. Patent No. 4,341,830 in which a tow of acrylic filaments is oxidized under tension, at a temperature of from 200° to 300°C, crimped in a stuffer box (thus imparting a pinch type crimp), made into staple fibers, spun into a yarn which is then knitted into a cloth panel and heat treated, ie. carbonized, in an inert atmosphere at a temperature of 1400°C. The so carbonized cloth panels are assembled into a stack and the stack placed into a carbon vapor furnace for deposition of carbon onto and into the stack. This treatment is carried out by passing a carbonaceous gas, i.e. methane, through the stack while inductively heating the stack to a temperature of 2000°C to cause carbon to be deposited onto and into the stack and thus produce a carbonaceous body having a matrix of the knitted panels. However, the yarn made by this process has been found, by Comparative Example A, to be very brittle and cannot be subjected to repeated acute angular stress bending such as would occur if the cloth panel were deknitted and carded, without severe breakage of the fibers.

GB-A-1190269 (corresponding to FR-A-1539755) discloses carbonizing a woven cloth of oxidized PAN or other polymeric fiber filament yarn. In a woven cloth the fibers are essentially linear and do not have a spring-like structural configuration (as defined above). There is no reference to disassembling the carbonized cloth into fibers except for extraction of fibers to test their physical properties.

US-A-4423675 discloses a carbon spring obtained by carbonizing a length of organic linear material in the form of a coiled spring. Specified organic linear materials include pitches and PAN. The material usually is extruded to a diameter of at least 100 micrometers and it appears to be essential that the coil is maintained under tension whilst being carbonized.

JP-A-44-2512 discloses the carbonation of Ishimeuchi or Admishiroushi woven cord or cloth formed from organic fiber yarn and subsequent removal of the warp fiber yarn to leave a resilient article. The resilience in said article arises from the arrangement of the constituent fiber yarns and not from the resilience of the fibers themselves. The fiber yarns have essentially linear portions between sharp return angle bends and hence the fibers do not have a spring-like configuration (as defined above). There is no reference to disassembling the resilient article into fibers.

JP-A-53-98423 discloses the formation of carbon fiber elements for use in incandescent lamps by carbonizing a coil of polymer fibers and subsequently graphitizing the set fiber coil. The coil is maintained under tension during carbonization and said carbonization is conducted at a temperature of at least 1500°C. The coil can be formed of a monofilament or a plurality, eg 400 to 1000, of monofilaments twisted together or formed into a cord.

US-A-4193252 (corresponding to JP-A-55-40885) discloses a method of producing carbon or graphite yarn from a fabric of knitted precursor yarn by carbonization, firing and graphitization of the yarn. The fabric can be deknitted after carbonization or firing and the deknitted yarn subjected to the subsequent heating step(s). Reference is made to use of twisted multi-ply yarn of the deknitted fibers obtained from the fired or graphitized fabric being of use as packing because of its resilience. The only exemplified precursor material is rayon and there is no reference to the carbonization of monofilaments or tows.

### Definitions

The term "fiber" or "filament" interchangeably refers to a fine threadlike body or structure of a natural or synthetic material in the conventional usage. Included herein are filaments made by melt spinning a pitch based composition such as petroleum or coal tar, or fibers which are made by wet spinning a synthetic resinous material such as polyacrylonitrile.

The term "fiber assembly" as used herein refers to a multiplicity of filaments commonly referred to in the textile industry as a tow. Fiber assemblies are made of common polymeric textile fibers or filaments, but are also applicable to carbonaceous fibers or filaments which have been stablized and treated in accordance with the following teaching and examples.

The term "spring-like" "spring-like structure", or "spring-like structural configuration" are interchangeably used herein to designate a fiber or tow that is physically deformed from a substantially linear configuration into a coil-like, sinusoidal, or other multi-curvilinear form or configuration having no acute angular bends.

The term "tow" herein refers to an assembly of a plurality of continuous filaments in which the number of filaments are identified by the designation nK wherein n is a numerical value in increments of 1000 filaments.

The term "staple" refers to non-continuous fibers which may be "spun" into yarns.

The term "stabilized" herein applies for example to fibers or tows which have been oxidized at a specific temperature, typically less than about 250°C for PAN fibers or, in some instances, oxidized by chemical oxidants at lower temperatures.

The term "yarn" herein applies to a continuous strand of twisted fibers. The term "spun yarn" refers to a continuous strand of staple fibers which has been drafted, drawn and twisted into a yarn.

The term "carding" herein refers to a procedure in which fibers are combed or brushed with a toothed apparatus, e.g. a wire tooth brush, to effect at least a partial alignment of the fibers into an entangled web or sliver.

The term "garnetted" herein refers to a process for reducing various textile waste materials to fiber by passing them through a machine called a garnett, which is similar to a card.

The term "knitting" herein includes single Jersey knit, Rib knit, Pearl knit, Interlock knit, Double knit, and similar methods of knitting a fiber, yarn or tow into a cloth.

The term "reversible deflection" or "working deflection" is used herein as it applies to a helical or sinusoidal compression spring to mean the extent, expressed as a ratio of extended to free spring length, to which a spring can repeatedly be extended and, on release of the extending force, return to its original (ie. free) length. Particular reference is made to the publication "Mechanical Design - Theory and Practice", MacMillan Publ. Co., 1975, pp 719 to 748; particularly Section 14-2, pages 721-24.

"Hooke's Law" herein refers to the stress applied to stretch or compress a body which is proportional to the strain or alteration in length so provided, as long as the limit of elasticity is not exceeded.

Carbonaceous precursor starting materials which have the capability of forming the spring-like structural configuration carbonaceous fiber of the invention are selected from starting materials such as pitch (petroleum or coal tar), polyacetylene, polyacrylonitrile (PANOX or GRAFIL), polyphenylene, polyvinylidene chloride (SARAN), and the like. GRAFIL, PANOX and SARAN are Trade Marks.

Preferred precursor materials are prepared by melt spinning or wet spinning in a manner to yield a monofilament or multi-filament assembly. The filaments are stabilized and then converted into a tow, or a woven cloth or knitted cloth by any of a number of commercially available techniques.

According to a first aspect of the present invention, there is provided a partially carbonized or substantially completely carbonized fiber derived from a continuous precursor fiber or tow of a stabilized, carbonaceous precursor material, said precursor fiber having a diameter of up to 30 micrometers, characterised in that the fiber has a permanently set multi-curvilinear structural configuration with no sharp bends and a reversible deflection ratio of greater than 1.2:1. Usually the fiber has a diameter of from 4 to 20 micrometers.

According to a second aspect of the present invention, there is provided a method of forming a fiber of the invention, comprising the steps of imparting and setting a multi-curvilinear shape having no sharp bends to a continuous precursor fiber or tow of a stabilized, carbonaceous material, said precursor fiber having a diameter of up to 30 micrometers; and heating the set fiber in a relaxed state under non-oxidizing conditions and at a temperature sufficient to impart a permanent setting of said shape to said fiber and at least partially carbonize the fiber.

In accordance with the present invention a unique article is prepared from such a carbonaceous precursor material which is made into a carbonaceous fiber or tow of fibers by stabilizing the fiber or tow and then providing it with a spring-like structural configuration, imparting to the fiber or tow flexible, resilient, elongatable and deflectable characteristics, without altering the spring-like configuration of the fiber over many cycles of elongation and contraction. Fibers made from PAN are generally oxidation stabilized at a temperature of from 200°C to 250°C and typically have a nominal diameter of from 10 to 20 micrometers. Fibers made from mesophase pitches are oxidation stabilized at a temperature of from 250° to 400°C, preferably at a temperature of from 300° to 390°C, as described in U.S. Patent No. 4005183. Fibers made from SARAN (Trade Mark) are stabilized by dehydrochlorination in which the SARAN fiber loses its thermoplastic nature and begins to take on a thermoset-like behavior. It will be understood that fibers having a somewhat larger diameter of, for example, 30 micrometers may be employed where stiffer fibers are desired, depending upon the particular end use to which such heavier and stiffer fibers are to be applied.

A multiplicity of continuous fibers are associated into a tow which is then stabilized by oxidation in conventional manner. The stabilized tow is thereafter, and in accordance with the present invention, formed into a coil-like structural configuration as, for example, by winding the tow on a cylindrical rod or mandrel, or is formed into a sinusoidal form or other multi-curvilinear form by knitting the tow into a fabric or cloth (recognizing that other fabric forming and coil forming methods can be employed). It is convenient to form the sinusoidal structure on a standard textile knitting machine (e.g. Flat bed knitting machine, or a tubular knitting machine) or in a rounded tooth gear-box that will not impart any sharp or acute angular bends to the fibers. The coil-like or sinusoidally shaped fiber, tow or the knitted cloth is thereafter heat treated in a relaxed state at a temperature of from 150°C to 1550°C. At a temperature of above about 250°C, the fiber, tow or cloth is heat treated in an inert atmosphere. If the desired end product requires subsequent mechanical treatment, ie. carding or deknitting of the fabric, it is preferable to subject the fiber, tow or cloth to a temperature below about 550°C in an inert atmosphere.

At a temperature of from 150°C to 550°C, the fibers are provided with a temporary set and have not yet acquired the high degree of brittleness associated with "graphite" fibers. However when the fibers are initally treated in the upper range of temperatures of from 550°C to 1550°C, the fibers are, ab initio, provided with a permanent set. Such permanent set is accompanied by some degree of brittleness which can lead to breakage of some fibers during subsequent treatment of the fibers.

It is especially critical that, if a spring- like configuration is imparted to the fiber or fiber tow by a rounded gear tooth crimp or by wrapping around a rod or mandrel, the fiber not be heated to a temperature above about 275°C, while under tension. Above this temperature, the fiber begins to lose weight and shrink in coilure diameter and the tension resulting from such shrinkage and weight loss causes non-annealable stress cracks and weak points in the fiber.

It is of course to be understood that the fiber or tow may be initially heat treated at the higher temperature range up to 1550°C so long as the heat treatment is conducted while the fiber is in a relaxed state (spring-like configuration) under an inert, non-oxidizing atmosphere. As a result of the higher temperature treatment, a permanent set spring-like structural configuration is imparted to the fiber. The resulting fibers or tow having such spring-like structural configuration may be used per se, or in the case of a knitted cloth, may be deknitted to form a sinusoidal or other multi-curvilinear tow. In either event the tow or the cloth per se may then be further subjected to a carding or garnetting operation or any of a number of other methods of mechanical treatment known in the art to create an entangled wool-like fluffy material in which, the fibers are separated into an entangled mass of fibers and in which the individual fibers retain their spring-like configuration.

For certain applications, it is preferred that the fibers of the invention have a density of less than 2.5 gm/cm³ and/or a Young's modulus of from 7 to 380 GPa.

The fibers, tow or the knitted cloth or the wool-like fluff produced by a heat treatment at a temperature of no higher than about 550°C, in a relaxed state (which has placed a temporary set spring-like configuration into the fibers, tow or thread) may then be further heat treated in a relaxed state and under a non-oxidizing atmosphere to a temperature of from 550°C to 1500°C to impart a permanent set, spring-like structural configuration to the fiber. At a temperature above 1550°C and up to about 3000°C, various lower degrees of electrical resistivity are imparted to the fibers, such resistivity being preferably less than about 10¹⁰ ohm-cm. In the case of PAN fibers, the diameter of the fibers is reduced when treated at a higher temperature up to about 1550°C. Although higher temperature treatment results in a gradually increasing brittleness, the fibers still retain their spring-like configuration. The precursor materials are of a nature believed to lose their non-carbon moieties upon heating and form a conjugated bond structure within the carbon to carbon backbones which are believed to convert to an aromatic, fused, ring-like form.

With careful handling and with improved handling techniques, brittle fibers produced at the higher temperatures of above 1000°C may still be useful as, for example, a structural reinforcement material for various synthetic resinous materials, as a filler material for rendering synthetic resinous materials antistatic, as electrical conductors (e.g. automobile ignition systems), as a thermal insulating material, or the like.

The stabilized fibers or tow, when heat-set into the desired spring-like structural configuration, e.g. by knitting, and thereafter heating in a relaxed state at a temperature of from 550°C to 1550°C retain their resilient and reversible, deflectable characteristics in accordance with Hooke's Law. If the tow has been knitted and heat treated in a relaxed state at a temperature between 550°C and 1000°C to "perm-set" the spring-like configuration in the tow, it may then be deknitted, carded, garnetted or otherwise mechanically treated to convert the deknitted tow to an entangled wool-like fluffy material which still retains a resilience similar to that found in wool.

A predetermined length of fiber or tow made into a spring-like structural configuration in accordance with the above described manner will exhibit a reversible deflection in excess of 1.2 times, generally greater than twice, of its relaxed, non-elongated, spring-like configuration. Stated another way, a fiber or tow which has been provided with a permanently set spring-like configuration can be stretched or elongated to a length of at least 1.2 times of its coiled, i.e. contracted, relaxed spring-like structural configuration length. By controlling the structural configuration, e.g. by controlling the knitting parameters such as the number of loops per unit length or the number of turns on a rod or mandrel, it is of course understood that a greater extension or elongation of the spring-like fiber or tow is possible. The tightness or looseness of the non-linear, coil or curl in the fiber, e.g. the loops per centimeter in a knitted cloth, therefor governs the extent of the elongation of the spring-like fiber or tow. Thus, the reversible deflection could be much greater than twice the length of a fiber or tow when in a relaxed state, spring-like configuration.

In a preferred embodiment, an assembly, e.g. a bundle of fibers is obtained, by spinning a carbonaceous precursor material into a fiber, stabilizing the fiber, assembling a multiplicity of mono-filaments or fibers into a tow, and knitting the tow into a cloth. After knitting, the fibers in the cloth are "set", i.e. temporarily formed into a coil-like or sinusoidal structure, by treating the knitted cloth at a temperature of from 150°C to 550°C. Preferably, the fibers in the knitted cloth are formed into a permanently set, spring-like structure at a temperature of from 550°C to 1550°C and most preferably at a temperature of less than 1000°C, under an inert atmosphere and in a relaxed condition. The fibers in the knitted cloth may then be carbonized at a temperature in excess of 1000°C to impart other desirable properties into the fibers, noted hereinabove.

Likewise, if a wool-like fluff is desired, the fiber tow having the spring-like configuration or even the knitted fabric, may be carded, garnetted, or otherwise mechanically treated either before or after treatment at a temperature of less than 1550°C, preferably less than 1000°C, and most preferably at a temperature of below about 650°C, when preparing a wool-like, fluffy material. If a higher electrical conductivity in a fiber is desired, the perm set (550°C to 1000°C) fiber, tow or cloth can be further heat treated to a temperature above 1000°C, e.g. up to 3000°C. As previously noted, fibers treated at a temperature above 1550°C become extremely brittle and do not readily lend themselves to a deknitting, carding or garnetting treatment. Accordingly, such carding and/or garnetting treatment should be accomplished prior to heat treatment to temperatures up to 1550°C for continuous fiber or fiber tows.

Fibers made from carbonaceous precursor materials normally have a surface area of from 0.5 to 1600 m²/gm, preferably less than 15m²/gm when produced according to the procedures set forth above. However, it is known that such fibers can have imparted to them a surface area of greater than this by rapidly heating the fibers to a high temperature thereby converting the non-carbon moieties to gases which, on leaving the fiber, disrupt the surface. Other techniques known in the art for producing high surface area, high porousity fibers include oxidation of the fiber surface. Such high porousity fibers can be prepared from the materials of the present invention by the same techniques after the spring-like structural configuration has been imparted into the fibers.

It is also to be understood that after formation of the spring-like structural configuration into the fiber, the continuous fibers or tows may be chopped into discrete lengths and made into non-woven products employing present day techniques for preparing such non-woven products.

Exemplary of the products which can be produced by the technique of the present invention are set forth in the following examples:

### Example 1

An oxidation (at a temperature of about 250°C) stabilized polyacrylonitrile PANOX (R.K. Textiles) continuous 3K or 6K tow (ie 3000 - 6000 fibers per tow) having nominal single fiber diameters of 12 micrometers, was knitted on a flat bed knitting machine into a cloth having from 3 to 4 loops per centimeter. Portions of this cloth were heat set at the temperatures set forth in Table I over a 6 hour period and under an inert atmosphere of nitrogen. When the cloth was deknitted, it produced a tow which had an elongation or reversible deflection ratio of greater than 2:1. The deknitted tow was cut into various lengths of from 5 to 25 cm, and fed into a Platts Shirley (Trade Mark) Analyzer. The fibers of the tow were separated by a carding treatment into a wool-like fluff, that is to say, the resulting product resembled an entangled wool-like mass or fluff in which the fibers had a high interstitial spacing and a high degree of interlocking as a result of the coiled and spring-like configuration of the fibers. The fiber lengths of each such treatment were measured and the results of these measurements set forth in Table I.

### Example 2

A fabric was knitted from a 3K or 6K PANOX (R.K. Textiles) continuous stabilized filament tow on a Singer flat bed knitting machine and heat treated at the temperatures set forth in Table II and under an inert atmosphere of nitrogen. The fabric was then deknitted and the tow having a spring-like structural configuration fed directly into a carding machine. The resulting wool-like mass was collected onto a rotating drum and had sufficient integrity to enable it to be easily handled. The length of the fibers ranged from 2 to 15 cm. The wool-like mass treated at a temperature of 950°C was highly conductive and had a resistance of less than 75 ohms at any probe length taken at widely separated distances up to 60 cm in the wool-like mass.

### Example 3

A 3K PANOX stabilized tow was knitted on a Singer flat bed knitting machine at a rate of 4 stitches/cm and was then heat treated at a temperature of 950°C and under an inert atmosphere of nitrogen. The cloth was deknitted and the tow (which had a coil elongation or reversible deflection ratio of greater than 2:1) cut into 7.5 cm lengths. The cut yarn was then carded on a Platt Minature Carding machine to produce a wool-like fluff having fibers ranging from 3.5 to 6.5 cm in length with an average length of about 5 cm. The wool-like fluff had a high electrical conductivity over any length of up to 60 cm tested.

### Example 4

In a similar manner to Example 3 a portion from the same knitted cloth was heat treated at a temperature of 1550°C and under an inert atmosphere of nitrogen. The cloth itself and the deknitted tow had a very high electrical conductivity. On carding 15 cm lengths of cut tow, a fluff was obtained which had fibers of lengths 2.5 to 9.5 cm with average lengths of 5 cm. Thus, carding of a deknitted, continuous filament tow, fabric which has been subjected to a temperature of above 1000°C is still capable of producing a wool-like fluffy product.

### Comparative Example A

A staple 2 ply singles 10's stabilized polyacrylonitrile PANOX yarn was knitted into a tubular sock at a rate of 4 loops per cm and thereafter heat treated at a temperature of 1550°C under an inert atmosphere of nitrogen and the yarn was then cut into 10 cm lengths. The cut yarn was carded in a carding machine. The resulting product was collected with difficulty. Only short fibers having a length of from 0.5 to 1.25 cm were obtained along with a high level of dust. The difficulty of fiber recovery resulted from the high degree of twist and fiber entanglement which is typically found in spun yarns. Similar results were obtained when this example was repeated starting with a similar spun yarn sample of Grafil-01 obtained from Hysol-Grafil Ltd., Coventry, England.

### Example 5

A series of runs were made to determine the effect various heat treatment temperatures had on the fibers. A significant property was the specific resistivity of the fibers. To determine such property, numerous samples of an oxidation stabilized polyacrylonitrile yarn having a density of from 1.35 to 1.38 g/cm³ yarn was assembled into 3K and 6K tows. The tows (identified as PANOX and manufactured by RK Textiles of Heaton-Norris, Stockport, England), were knitted into a plain jersey flat cloth having from 3 to 4 stitches per cm, respectively. The cloth was thereafter heat treated at various temperatures under an oxygen-free nitrogen pad in an incremental heat control quartz tube furnace. The temperature of the furnace was gradually increased from room temperature to about 550°C over a three hour period with the higher temperatures being achieved by 50°C increments every 10-15 min. The material was held at the desired temperature for about 1 hour, the furnace opened and allowed to cool while purging with nitrogen. Representative of the furnace temperatures at the above preset incremental temperature schedule is that for a 6K yarn and shown in Table III following:

**TABLE III**

| Time | Temp. °C |
|---|---|
| 0720 | 200 |
| 0810 | 270 |
| 0820 | 300 |
| 0830 | 320 |
| 0840 | 340 |
| 0850 | 360 |
| 0900 | 370 |
| 0905 | 380 |
| 0935 | 420 |
| 0950 | 450 |
| 1005 | 500 |
| 1010 | 550 |
| 1025 | 590 |
| 1035 | 650 |
| 1045 | 700 |
| 1100 | 750 |
| 1400 | 750 |

The specific resistivity of the fibers was calculated from measurements made on each sample using a measured average of six measurements, one made from fibers removed at each corner of the sample and one made from fibers removed from each edge approximately at the middle of the sample. The results are set forth in Table IV following:

**TABLE IV**

| Final Temp. in °C | % wt. loss | Log Specific Resistivity |
|---|---|---|
| 500 | - | 4.849 |
| 550 | 33 | - |
| 600 | - | 2.010 |
| 650 | 34 | - |
| 700 | - | - |
| 750 | 37 | - 1.21 |
| 850 | 38 | - 2.02 |
| 900 | 42 | - 2.54 |
| 950 | 45 | - 2.84 |
| 1000 | 48 | - 3.026 |
| 1800 | 51 | - 3.295 |

The carbonized and permanently set fibers of the invention, when treated at temperatures sufficiently high to render the fibers electrically conductive and yet sufficiently low where the fibers still exhibit resilient, flexible, and non- brittle characteristics, are particularly suitable for blending with standard carpet fibers or yarn to produce a yarn having static dissipation properties. Such a carpet/yarn blend may incorporate at least 0.25 weight percent carbonized fibers in the carpet yarn. The weight ratio of synthetic carpet fibers to carbonized fibers is preferably greater than 100:1 to 200:1. A carpet employing the carbonized fibers of the invention exhibited static discharge properties to 0 percent of an applied electrostatic charge in less than 1 second.

### Example 6

Monsanto 1879 nylon (trilobal) staple was blended with 0.5 percent by weight of a conductive fiber prepared in accordance with the present invention. The conductive fiber was prepared by heating an oxidatively stabilized polyacrylonitrile multifilament fiber tow which had been knitted into a cloth, heat treated at about 1500°C, deknitted and cut into staple approximately 18 cm in length. The blended staple was carded and the resulting sliver was pin drafted three times, recombination ratios were 10:1, 3:1, and 5.1, respectively. The resulting drafted sliver was spun into a single ply yarn with an average twist of about 4.75. The majority of the carbonaceous fiber was broken into lengths much smaller than the original 18 cm lengths, resulting in a large loss of carbonaceous fiber from that originally included in the singles spinning process. The resulting carbonaceous fiber containing singles yarn was plied with a nylon yarn made in the same fashion but containing no carbonaceous fiber. The 3.00/2 ply yarn which was heat set on a Suessen (Trade Mark) heat setting apparatus was thereafter tufted into a 1/8 inch (3 mm) gauge, 27 on (765 gm), 9.5 mm pile height carpet (a cut loop form) with approximately 3 stitches per cm. The ratio of carbonaceous fiber to yarn containing no carbonaceous yarn in the tufting operation was 1:5 respectively. A portion of the carpet was backed with a commercial non-conductive latex carpet backing. The resulting carpet was tested for static discharge properties by charging the carpet to 5000 volts while in an atmosphere having a relative humidity of less than 20 percent. The static charge was dissipated to 0 percent of original charge in less than one second, and some of the samples discharged in less than 1/2 second. The standard for the industry is a discharge to 0 percent in 2 seconds or less.

This example illustrates that temperatures above about 1000°C can be employed in heat-setting the spring-like structural configuration into the carbonaceous fiber tow, but that at temperatures above 1000°C much embrittlement occurs and the fibers resulting were inefficiently used, being lost as short fibers not incorporated into the yarn when drafted with normal carpet staple to prepare singles.

### Example 7

In another example 100 grams of the same precursor acrylonitrile fiber tow as described in Example 6 was used. However, the precurser fiber was heat treated after knitting at a temperature of 950°C. All other aspects of handling the carbonaceous material were the same. The carbonized fiber was blended with 45 kg of the Monsanto 1879 nylon yarn as in Example 6. The resulting yarn contained 0.02 percent carbonized fibers which were substantially evenly distributed throughout the yarn. The yarn was tufted to prepare a carpet in a similar manner to Example 6. Thus, each tufted end has the carbonized fibers. Results were similar to the results obtained in Example 6.

Knitted fiber tows which have been heat treated to a temperature above 1000°C, and thus been rendered electrically conductive, have also found special utility in the manufacture of electrodes for a non-aqueous secondary energy storage device such as described in GB-A-2150741.

### Example 8

In another experiment tows made by deknitting a flat stock cloth in which the tow was a stabilized polyacrylonitrile precursor of the indicated filament count which had been heat-set at the indicated temperatures prior to deknitting. Tow lengths were measured for resilient deflection by adding known weights to the tow portion and the intermediate and the final deformations as well as the final non-resilient elongation deflection measured. The results are set forth in Table V.

### Comparative Example B

To illustrate the effect of tension on the fibers during setting of the spring-like configuration, a 6K tow of Panox continuous fibers was roll-wrapped onto a 8 mm quartz rod. The wound tow was heat treated according to the schedule as set forth in Example 5, Table III to a final temperature of 300°C while holding the ends of the wrapped tow secure. The heat treatment set a spring-like configuration into the tow. However, the fibers were very stiff and the tow was removed from the rod with difficulty. Many of the fibers broke on removal. This tow did not have the same resilience as tows which had been heat set in a relaxed knitted configuration. If the same procedure is employed but the spring-like tow is heated to a temperature of 350°C much greater breakage occurs even before removal.

The latter procedure was repeated and the heat treated material (350°C) after being carefully removed from the rod, was heated while in a relaxed state slowly to about a temperature of 650°C to determine whether any annealing would occur. None did. The resultant coil was brittle and had no resiliency.

However, if the wrapped coiled tow was removed from the rod prior to reaching 275°C and a smaller diameter rod inserted to maintain the integrity of the spring-like shape, heating in this "relaxed" state resulted in a spring like tow having substantially the same properties as the aforedescribed deknitted tows.

## Claims

1. A partially carbonized or substantially completely carbonized fiber derived from a continuous precursor fiber or tow of a stabilized, carbonaceous precursor material, said precursor fiber having a diameter of up to 30 micrometers, characterised in that the fiber has a permanently set multi-curvilinear structural configuration with no sharp bends and a reversible deflection ratio of greater than 1.2:1.

2. A fiber as claimed in Claim 1, wherein said fiber has been stabilized by oxidation.

3. A fiber as claimed in Claim 2, wherein said precursor fiber is a polyacrylonitrile fiber.

4. A fiber as claimed in Claim 3, wherein the log specific resistivity of said carbonized fiber is greater than -2.84.

5. A fiber as claimed in Claim 1, wherein said precursor fiber is a polyvinylidene chloride fiber stabilized by dehydrochlorination.

6. A fiber as claimed in any one of the preceding claims, wherein said diameter is from 4 to 20 micrometers.

7. A fiber as claimed in any one of the preceding claims, wherein said reversible deflection ratio is greater than 2:1.

8. A fiber as claimed in any one of the preceding claims, having a specific electrical resistivity of less than 10¹⁰ ohm-cm.

9. A fiber as claimed in any one of the preceding claims, wherein the density of the fiber is less than 2.5 gm/cm³.

10. A fiber as claimed in any one of the preceding claims, wherein the Young's modulus of the fiber is from 7 GPa to 380 GPa.

11. A fiber as claimed in any one of the preceding claims, wherein the surface area of said carbonized fiber is from 0.5 to 1600 m²/gm.

12. A fiber as claimed in Claim 11, wherein said surface area is 0.5 to 15 m²/gm.

13. A wool-like fluff comprising an entangled multiplicity of carbonized fibers as claimed in any one of the preceding claims.

14. A fluff as claimed in Claim 13, wherein the electrical resistance at a probe distance of 60 cm measured across the wool-like fluff is less than 75 ohms.

15. An article comprising carbonized fibers as claimed in any one of Claims 1 to 12.

16. An article as claimed in Claim 15, wherein said article is non-woven.

17. A method of forming a fiber as claimed in Claim 1, comprising the steps of imparting and setting a multi-curvilinear shape having no sharp bends to a continuous precursor fiber or tow of a stabilized, carbonaceous material, said precursor fiber having a diameter of up to 30 micrometers; and heating the set fiber in a relaxed state under non-oxidizing conditions to a temperature sufficient to impart a permanent setting of said shape to said fiber and at least partially carbonize the fiber.

18. A method as claimed in Claim 17, including the step of heating said shaped stabilized fiber in a relaxed state under non-oxidizing conditions to a temperature of from 150°C to 550°C to impart a temporary setting of said shape to the fiber.

19. A method as claimed in Claim 17 or Claim 18, wherein said shaped stabilized fiber is heated to a temperature of from 550°C to 1550°C under non-oxidizing conditions to impart a permanent setting of said shape.

20. A method as claimed in any one of Claims 17, 18 and 19, wherein a multiplicity of said stabilized precursor fibers are assembled into a fiber tow, said multi-curvilinear shape is imparted to said fiber tow, and said shaped fiber tow is heated in a relaxed state under non-oxidizing conditions to permanently set said shape and at least partially carbonize the fibers tow.

21. A method as claimed in Claim 20, wherein the stabilized fiber tow is wound around a cylindrical rod or mandrel, the wound fiber tow is heated to a temperature of from 150°C to 300°C in a non-oxidizing atmosphere, the fiber tow is unwound from the cylindrical rod or mandrel, and heated in a relaxed condition in an inert atmosphere, to a temperature of from 550°C to 1550°C.

22. A method as claimed in any one of Claims 17 to 20, wherein said multi-curvilinear shape is imparted by knitting the fiber into a cloth, said cloth is heated under non-oxidizing conditions to a temperature at least sufficient to impart a temporary setting of the shape of the knitted fiber and the set cloth deknitted.

23. A method as claimed in Claim 22, wherein the knitted cloth is heated to a temperature of from 150°C to 550°C to impart a temporary set to the fibers in the cloth, and the temporary set cloth is deknitted.

24. A method as claimed in Claim 23, wherein the fibers from the deknitted cloth are heated to a temperature of from 550°C to 1000°C to permanently set the fibers.

25. A method as claimed in any one of Claims 17 to 24, wherein the set fiber is mechanically treated to form a wool-like fluff.

26. A method as claimed in any one of Claims 17 to 25, wherein the shaped fiber is heated at a temperature of less than 1000°C to render it electrically conductive.

27. A method as claimed in any one of Claims 17 to 26, wherein the shaped fiber is heated to a temperature of greater than 1000°C to render it more highly electrically conductive.

28. A method as claimed in Claim 27, wherein the electrically conductive fiber is incorporated into a synthetic resinous material.

29. A method as claimed in any one of Claims 17 to 28, wherein the carbonized fiber is heated in a non-oxidizing atmosphere at a temperature up to 3000°C to render the fiber electrically conductive.

30. A method as claimed in any one of Claims 17 to 29, wherein the precursor fiber is as defined in any one of Claims 2 to 6.

31. A method as claimed in any one of Claims 17 to 30, wherein the process conditions are such as to provide a fiber as defined in any one of Claims 7 to 12.

## Patentansprüche

1. Teilweise carbonisierte oder im wesentlichen vollständig carbonisierte Faser, die von einer kontinuierlichen Vorläuferfaser oder einem Kabel aus einem stabilisierten, kohlenstoffhaltigen Vorläufermaterial stammt, wobei die Vorläuferfaser einen Durchmesser bis zu 30 Mikrometer aufweist,
**dadurch gekennzeichnet,**
daß die Faser eine dauerhaft fixierte, mehrfach krummlinige strukturelle Konfiguration ohne scharfe Biegungen und ein reversibles Auslenkungsverhältnis von mehr als 1,2:1 aufweist.

2. Faser nach Anspruch 1, worin die Faser durch Oxidation stabilisiert worden ist.

3. Faser nach Anspruch 2, worin die Vorläuferfaser eine Polyacrylnitrilfaser ist.

4. Faser nach Anspruch 3, worin der Logarithmus des spezifischen Widerstands der carbonisierten Faser mehr als -2,84 ist.

5. Faser nach Anspruch 1, worin die Vorläuferfaser eine durch Dehydrochlorierung stabilisierte Polyvinylidenchloridfaser ist.

6. Faser nach einem der vorhergehenden Ansprüche, worin der Durchmesser von 4 bis 20 Mikrometer ist.

7. Faser nach einem der vorhergehenden Ansprüche, worin das reversible Auslenkungsverhältnis größer als 2:1 ist.

8. Faser nach einem der vorhergehenden Ansprüche mit einem spezifischen elektrischen Widerstand von weniger als 10¹⁰ Ohm-cm.

9. Faser nach einem der vorhergehenden Ansprüche, worin die Dichte der Faser weniger als 2,5 g/cm³ ist.

10. Faser nach einem der vorhergehenden Ansprüche, worin der Young'sche Modul der Faser von 7 GPa bis 380 GPa ist.

11. Faser nach einem der vorhergehenden Ansprüche, worin die Oberfläche der carbonisierten Faser von 0,5 bis, 1600 m²/g ist.

12. Faser nach Anspruch 11, worin die Oberfläche 0,5 bis 15 m²/g ist.

13. Wolleartiger Flaum, umfassend eine verwickelte Vielzahl von carbonisierten Fasern nach einem der vorhergehenden Ansprüche.

14. Flaum nach Anspruch 13, worin der elektrische Widerstand bei einer Meßstrecke von 60 cm, gemessen über den wolleartigen Flaum, weniger als 75 Ohm ist.

15. Gegenstand, der carbonisierte Fasern nach einem der Ansprüche 1 bis 12 enthält.

16. Gegenstand nach Anspruch 15, worin der Gegenstand vliesartig ist.

17. Verfahren zur Herstellung einer Faser nach Anspruch 1, umfassend die Schritt des Einführens und Fixierens einer mehrfach krummlinigen Form ohne scharfe Biegungen in eine kontinuierliche Vorläuferfaser oder ein Kabel aus einem stabilisierten, kohlenstoffhaltigen Material, wobei die Vorläuferfaser einen Durchmesser von bis zu 30 Mikrometer aufweist, und des Erhitzens der fixierten Faser in einem entspannten Zustand unter nicht oxidierenden Bedingungen auf eine Temperatur, die ausreicht, um eine dauerhafte Fixierung der Form in die Faser einzuführen und die Faser mindestens teilweise zu carbonisieren.

18. Verfahren nach Anspruch 17, umfassend den Schritt des Erhitzens der geformten, stabilisierten Faser in einem entspannten Zustand unter nicht oxidierenden Bedingungen auf eine Temperatur von 150°C bis 550°C, um eine zeitweise Fixierung der Form in die Faser einzuführen.

19. Verfahren nach Anspruch 17 oder 18, worin die geformte, stabilisierte Faser auf eine Temperatur von 550°C bis 1550°C unter nicht oxidierenden Bedingungen erhitzt wird, um eine dauerhafte Fixierung der Form einzuführen.

20. Verfahren nach einem der Ansprüche 17, 18 und 19, worin eine Vielzahl der stabilisierten Vorläuferfasern zu einem Faserkabel zusammengefügt werden, die mehrfach krummlinige Form in das Faserkabel eingeführt wird und das geformte Faserkabel in einem entspannten Zustand unter nicht oxidierenden Bedingungen erhitzt wird, um die Form dauerhaft zu fixieren und mindestens teilweise das Faserkabel zu carbonisieren.

21. Verfahren nach Anspruch 20, worin das stabilisierte Faserkabel um einen zylindrischen Stab oder eine Spindel gewickelt wird, das gewickelte Faserkabel auf eine Temperatur von 150°C bis 300°C in einer nicht oxidierenden Atmosphäre erhitzt wird, das Faserkabel vom zylindrischen Stab oder der Spindel abgewickelt und in einem entspannten Zustand in einer inerten Atmosphäre auf eine Temperatur von 550°C bis 1550°C erhitzt wird.

22. Verfahren nach einem dar Ansprüche 17 bis 20, worin die mehrfach krummlinige Form durch Wirken der Faser zu einem Stoff eingeführt wird, wobei der Stoff unter nicht oxidierenden Bedingungen auf eine Temperatur erhitzt wird, die mindestens ausreicht, um eine zeitweise Fixierung der Form in die gewirkte Faser einzuführen, und der fixierte Stoff entwirkt wird.

23. Verfahren nach Anspruch 22, worin der gewirkte Stoff auf eine Temperatur von 150°C bis 550°C erhitzt wird, um eine zeitweise Fixierung in die Fasern im Stoff einzuführen und der zeitweise fixierte Stoff entwirkt wird.

24. Verfahren nach Anspruch 23, worin die Fasern aus dem entwirkten Stoff auf eine Temperatur von 550°C bis 1000°C erhitzt werden, um die Fasern dauerhaft zu fixieren.

25. Verfahren nach einem der Ansprüche 17 bis 24, worin die fixierte Faser mechanisch behandelt wird, um einen wolleartigen Flaum zu bilden.

26. Verfahren nach einem der Ansprüche 17 bis 25, worin die geformte Faser bei einer Temperatur von weniger als 1000°C erhitzt wird, um sie elektrisch leitfähig zu machen.

27. Verfahren nach einem der Ansprüche 17 bis 26, worin die geformte Faser auf eine Temperatur von mehr als 1000°C erhitzt wird, um sie stärker elektrisch leitfähig zu machen.

28. Verfahren nach Anspruch 27, worin die elektrisch leitfähige Faser in ein synthetisches Harzmaterial eingebaut wird.

29. Verfahren nach einem der Ansprüche 17 bis 28, worin die carbonisierte Faser in einer nicht oxidierenden Atmosphäre bei einer Temperatur bis zu 3000°C erhitzt wird, um die Faser elektrisch leitfähig zu machen.

30. Verfahren nach einem der Ansprüche 17 bis 29, worin die Vorläuferfaser wie in einem der Ansprüche 2 bis 6 definiert ist.

31. Verfahren nach einem der Ansprüche 17 bis 30, worin die Arbeitsbedingungen so sind, um eine Faser, wie in einem der Ansprüche 7 bis 12 definiert, zu liefern.

## Revendications

1. Fibre partiellement carbonisée ou quasiment carbonisée en totalité dérivée d'une fibre ou d'une mèche précurseur continue d'un matériau carboné stabilisé précurseur, ladite fibre précurseur ayant un diamètre allant jusqu'à 30 micromètres, caractérisée en ce que la fibre a une configuration structurelle, fixée de façon permanente, muticurvilinéaire sans aucun pli aigu et un rapport de déflexion réversible supérieur à 1,2/1.

2. Fibre selon la revendication 1, dans laquelle ladite fibre a été stabilisée par oxydation.

3. Fibre selon la revendication 2, dans laquelle ladite fibre précurseur est une fibre de polyacrylonitrile.

4. Fibre selon la revendication 3, dans laquelle le log de la résistivité spécifique de ladite fibre carbonisée est supérieur à -2,84.

5. Fibre selon la revendication 1, dans laquelle ladite fibre précurseur est une fibre de chlorure de polyvinylidène stabilisée par déshydrochloration.

6. Fibre selon l'une quelconque des revendications précédentes, dans laquelle ledit diamètre est de 4 à 20 micromètres.

7. Fibre selon l'une quelconque des revendications précédentes, dans laquelle ledit rapport de déflexion réversible est supérieur à 2/1.

8. Fibre selon l'une quelconque des revendications précédentes, ayant une résistivité électrique spécifique inférieure à 10¹⁰ ohm-cm.

9. Fibre selon l'une quelconque des revendications précédentes, dans laquelle la densité de la fibre est inférieure à 2,5 g/cm³.

10. Fibre selon l'une quelconque des revendications précédentes, dans laquelle le module de Young de la fibre est de 7 GPa à 380 GPa.

11. Fibre selon l'une quelconque des revendications précédentes, dans laquelle la surface spécifique de ladite fibre carbonisée est de 0,5 à 1 600 m²/g.

12. Fibre selon la revendication 11, dans laquelle ladite surface spécifique est 0,5 à 15 m²/g.

13. Peluche analogue à de la laine comprenant une multiplicité emmêlée de fibres carbonisées selon l'une quelconque des revendications précédentes.

14. Peluche selon la revendication 13, dans laquelle la résistance électrique mesurée à travers la peluche analogue à de la laine à une distance d'épreuve de 60 cm est inférieure à 75 ohms.

15. Article comprenant des fibres carbonisées selon l'une quelconque des revendications 1 à 12.

16. Article selon la revendication 15, dans lequel ledit article est non tissé.

17. Procédé de formation d'une fibre selon la revendication 1, comprenant les étapes consistant à communiquer et à fixer une forme multicurvilinéaire n'ayant aucun pli aigu à une fibre ou mèche précurseur continue d'un matériau stabilisé carboné, ladite fibre précurseur ayant un diamètre allant jusqu'à 30 micromètres; et à chauffer la fibre fixée à l'état détendu dans des conditions non-oxydantes à une température suffisante pour communiquer une fixation permanente de ladite forme à ladite fibre et à carboniser au moins partiellement la fibre.

18. Procédé selon la revendication 17, comprenant l'étape de chauffage de ladite fibre stabilisée formée à l'état détendu dans des conditions non-oxydantes à une température allant de 150°C à 550°C pour communiquer une fixation temporaire de ladite forme à la fibre.

19. Procédé selon la revendication 17 ou 18, dans lequel ladite fibre stabilisée formée est chauffée à une température allant de 550°C à 1550°C dans des conditions non-oxydantes pour communiquer une fixation permanente de ladite forme.

20. Procédé selon l'une quelconque des revendications 17, 18 et 19, dans lequel une multiplicité desdites fibres précurseurs stabilisées sont assemblées dans une mèche de fibres, ladite forme multicurvilinéaire est communiquée à ladite mèche de fibres, et ladite mèche de fibres formée est chauffée à l'état détendu dans des conditions non-oxydantes pour fixer de façon permanente ladite forme et carboniser au moins partiellement la mèche de fibres.

21. Procédé selon la revendication 20, dans lequel la mèche de fibres stabilisée est enroulée autour d'une baguette ou d'un mandrin cylindrique, la mèche de fibres enroulée est chauffée à une température allant de 150°C à 300°C dans une atmosphère non-oxydante, la mèche de fibres est déroulée de la baguette ou du mandrin cylindrique, et chauffée à l'état détendu dans une atmosphère inerte à une température allant de 550°C à 1 550°C.

22. Procédé selon l'une quelconque des revendications 17 à 20, dans lequel ladite forme multicurvilinéaire est communiquée en tricotant la fibre en un tissu, ledit tissu est chauffé dans des conditions non-oxydantes à une température au moins suffisante pour communiquer une fixation temporaire de la forme de la fibre tricotée et le tissu fixé est détricoté.

23. Procédé selon la revendication 22, dans lequel le tissu tricoté est chauffé à une température allant de 150°C à 550°C pour communiquer une fixation temporaire aux fibres dans le tissu, et le tissu fixé temporairement est détricoté.

24. Procédé selon la revendication 23, dans lequel les fibres du tissu détricoté sont chauffées à une température allant de 550°C à 1 000°C pour fixer de façon permanente les fibres.

25. Procédé selon l'une quelconque des revendications 17 à 24, dans lequel la fibre fixée est traitée mécaniquement pour former une peluche analogue à de la laine.

26. Procédé selon l'une quelconque des revendications 17 à 25, dans lequel la fibre formée est chauffée à une température inférieure à 1000°C pour la rendre conductrice de l'électricité.

27. Procédé selon l'une quelconque des revendications 17 à 26, dans lequel la fibre formée est chauffée à une température supérieure à 1000°C pour la rendre plus fortement conductrice de l'électricité.

28. Procédé selon la revendication 27, dans lequel la fibre conductrice de l'électricité est incorporée dans une résine synthétique.

29. Procédé selon l'une quelconque des revendications 17 à 28, dans lequel la fibre carbonisée est chauffée dans une atmosphère non-oxydante à une température allant jusqu'à 3 000°C pour rendre la fibre conductrice de l'électricité.

30. Procédé selon l'une quelconque des revendications 17 à 29, dans lequel la fibre précurseur est définie comme dans l'une quelconque des revendications 2 à 6.

31. Procédé selon l'une quelconque des revendications 17 à 30, dans lequel les conditions du traitement sont telles qu'il est fourni une fibre définie comme dans l'une quelconque des revendications 7 à 12.
